

1

2,931,749

**BONDED NON-WOVEN FIBROUS PRODUCTS  
AND METHODS FOR MAKING THEM**

Benjamin B. Kine and Nathaniel A. Matlin, Levittown, Pa., assignors to Rohm & Haas Company, Philadelphia, Pa., a corporation of Delaware

No Drawing. Application August 13, 1956  
Serial No. 603,832

15 Claims. (Cl. 154—101)

This invention relates to bonded non-woven fibrous or filamentous products having a carded fiber structure or comprising fibrous mats in which the fibers or filaments are distributed haphazardly or in random array. The invention also relates to methods for producing the bonded non-woven fibrous products or shaped articles therefrom. The bonded non-woven fibrous products are useful in the production of articles of either flat or three-dimensional shape, including insulating material and the like as will be described more particularly hereinafter.

Hereinafter, the expression "random array" is intended to include the array of fibers in a carded web wherein partial orientation is frequently present as well as other arrays in which the fibers are in a completely haphazard distributional relationship.

Heretofore binders of natural rubber latex and aqueous dispersions of synthetic rubbers, such as butadiene copolymerized with styrene, acrylonitrile, and so on have been suggested as binders for bonding the fibers in non-woven fabric structures; but these materials have various disadvantages, among which is the tendency to produce an off-white appearance or cast to the bonded products, and this tendency is so strong it is difficult to overcome even by the use of optical bleaches or by the use of white pigments, such as titanium dioxide. These rubbery binders also produce a rubbery hand which appears to be the result of a complete suppression of the fibrous character insofar as the feel of the product is concerned. When binders of polyvinyl acetates, chlorides, or their copolymers are used, the hand becomes papery, by which is meant that the product has a crisp, brittle hand and conveys the impression of thinness and fragility. It also produces a noise on crumpling that is typical of papers. The application of thermoplastic polymers such as simple esters of acrylic or methacrylic acid produces products in which the binder remains permanently thermoplastic with consequent tendency to change when subjected to excessive temperatures. The simple acrylic and methacrylic acid esters are also characterized by relatively poor adhesion to hydrophobic types of fibers, such as nylon, vinyl resin fibers, cellulose esters and such polyesters as polyethylene glycol terephthalate. Furthermore, many of the binders heretofore employed, including the aqueous dispersions of rubber, synthetic rubbers, and acrylic esters, have a strong tendency to migrate to the surfaces of the fibrous products during drying of the products to which the dispersions have been applied.

It is an object of the present invention to provide fibrous products made with a binder which can be applied by way of an aqueous system without the disadvantages mentioned above that are characteristic of previously applied aqueous binder systems. A further object of the invention is to provide a bonded fibrous product of non-woven character in which the binder is adapted to be converted to an infusible and insoluble condition as by heating with or without the presence of a suitable catalyst as will be pointed out more particularly hereinafter. It is a further object of the present invention to produce

2

bonded fibrous products of non-woven character from fibers which are incapable of felting, whether of natural or synthetic origin, and especially those which, unlike wool, are of non-proteinaceous character and have relatively smooth surfaces extending longitudinally of the fibers, and because of these surface characteristics are incapable of being converted into a felted product by normal felting operations. A further object of the invention is to provide bonded fibrous products of non-woven character wherein the binder may be substantially uniformly distributed through the body of the structure and has reduced tendency to migrate preferentially to the surfaces of the structure. Other objects and advantages of the invention will be apparent from the description thereof hereinafter.

In a copending application Serial No. 474,264, filed December 9, 1954, in the hands of a common assignee, bonded fibrous products are obtained by treating a fibrous web or mat with an aqueous dispersion of a polyvalent metal compound, yielding polyvalent metal ions, and of a water-insoluble linear copolymer of monoethylenically unsaturated monomeric units comprising 0.5 to 7 mole percent of units containing carboxyl (—COOH) groups, held in stable dispersed condition by means of a non-ionic emulsifier. On drying the treated fibrous product, the copolymer becomes cross-linked to insoluble and infusible condition by the polyvalent metal.

In accordance with the present invention, it has been discovered that solvent-resistant, heat-resistant bonded non-woven fibrous products can be obtained by the application of an aqueous dispersion of a water-insoluble linear copolymer, or salts thereof, of monoethylenically unsaturated monomeric units comprising 0.5 to 10 percent by weight of units containing carboxyl (—COOH) groups without a polyvalent metal compound provided the fibrous product, after application of the copolymer, is heated to a temperature between 110° C. and 350° C. or even as high as 400° C. for a period of time which may range from as short as a fourth of a minute at the higher temperature and as long as half an hour or more at the lower temperature, either with or without an auxiliary aminoplast of the type described more particularly hereinafter and an acidic catalyst therefor. Generally, baking at the temperatures mentioned increases the solvent-resistance and the heat-resistance of the copolymer adequately for many purposes, especially when the copolymer contains at least 2.5% by weight of dicarboxylic acid units, such as those obtained from itaconic acid, or at least 5% by weight of monocarboxylic acid units, such as those obtained from acrylic or methacrylic acid. When less than the minimum proportions of carboxylic acid units just specified are present, it is generally preferred to use an aminoplast along with the copolymer to enhance the resistance of the products to solvents and heat. Some enhancement of these properties is frequently obtained when an aminoplast is used in conjunction with copolymers containing carboxyl units in the higher portion of the broad range specified, but usually the aminoplast is unnecessary in these instances.

The copolymer may be applied in free acid form (—COOH groups) or in the form of an alkali metal salt, such as of sodium, potassium or lithium (e.g. —COONa groups), an ammonium salt (—COONH<sub>4</sub>) or a salt of a water-soluble amine, such as methylamine, diethylamine, triethylamine, mono-, di-, or tri-ethanolamine, morpholine, etc. Generally, it is desirable to apply the copolymer dispersion at a pH at least about 5 and preferably at a pH between 6 and 10.

One advantage of the present invention over the use of dispersions of the above-mentioned application Serial No. 474,264 is that emulsifiers of anionic type can be used as well as those of non-ionic type in making the

aqueous copolymer dispersion without encountering stability problems. The versatility of the binder used in the present invention is such as to be readily adapted to various methods of production of the fibrous products.

The bonding of the fibers is effected with a clear, substantially colorless binder which has good adhesion to all sorts of fibers and filaments and even to those of siliceous character including glass which, in the past, have been difficult to handle because of the difficulty of finding colorless binder materials which are adequately adhesive toward the siliceous material. The binders of the present invention are also substantially free of discoloration when subjected to elevated temperatures, such as those used for drying, fusing, or curing.

The copolymer used in the binder of the present invention contains a plurality of carboxyl (—COOH) groups either in free acid or salt form by which it is adapted to be insolubilized and rendered infusible on heating with or without an auxiliary aminoplast and suitable catalysts which are generally of acidic character. Hence, the cured or baked fibrous product provides improved resistance to laundering, dry-cleaning and spotting, to various chemicals, and to heat as compared to such aqueous systems as rubber latex or aqueous dispersions of synthetic rubbers or acrylic or vinyl esters, heretofore applied. The bonded fibrous products of the present invention can be heated to a much higher temperature than those of the prior art using the binders mentioned above without suffering discoloration, increase in stiffness or deleterious decomposition. They are characterized by excellent resistance to ironing in which operation they are not subject to tackiness as would be true of the thermoplastics heretofore used. The carboxyl groups apparently also provide a greater versatility of adhesion in that the binders of the present invention are characterized not only with good adhesion to hydrophilic fibers like cotton, regenerated cellulose rayons and the like, but they are also characterized by excellent adhesion to hydrophobic types of fibers, such as the nylons and especially the polyamide types, the vinyl resins such as copolymers of vinyl chloride with vinyl acetate or with acrylonitrile, polymers of 70 to 90% acrylonitrile with other monomers such as vinyl chloride, vinyl acetate, any of the vinyl pyridines such as 2-vinyl pyridine or mixtures of such auxiliary comonomers, polyesters such as poly(ethylene glycol terephthalate), and cellulose esters such as cellulose acetate, cellulose acetate propionate, cellulose acetate butyrate and so on. Because of the characteristic adhesion of the binder of the present invention to both hydrophilic and hydrophobic types of fibers, the fibrous products are characterized by excellent resistance to "pilling" and abrasion. The binder of the present invention is adapted to be dried and then cured to insoluble and infusible condition so that the bonds cannot be disturbed even under severe conditions of heat. The fibrous products using the binder of the present invention have the advantage also that they can be embossed durably in wet condition or during the first drying but before complete drying. This is evidenced by the fact that if the drying is effected on a suction screen through which the excess water is drained from the fibrous product, the pattern of the screen is permanently imparted to one face of the product and even calendering under normal procedures and temperatures does not destroy this pattern effect. While the binder may be preferentially applied, if desired, to portions of the fibrous product, such as one or both of the faces thereof, it is characteristic of the binder of the present invention that, if such preferential treatment is not desired, substantially uniform distribution may be obtained because of the reduced tendency of the binder after initial distribution throughout the body of the fibrous product to migrate to the surfaces thereof during drying. The binder of the present invention may also contain, besides the linear copolymer, thermosetting aminoplast condensates such as of urea or melamine or the like with formaldehyde and

the catalyst used for accelerating the condensation of the aminoplast to insoluble and infusible condition serves simultaneously and/or concurrently for the curing of the carboxylate-containing polymer to the insoluble and infusible condition.

5 The cured or insolubilized binders are unaffected by water or organic solvents, such as styrene, even at molding temperatures, whereby the bonded fibrous products are adapted to be used as molding preforms or molding 10 inserts for the production of molded articles from various thermosetting resins as will be pointed out in more detail hereinafter. The binders are also free of cold flow and are resistant to flow at elevated temperatures, whereby shifting of the fibers or filaments in the bonded products 15 is substantially completely prevented even at elevated temperatures during subsequent molding with such products being used as reinforcing inserts or preforms.

In accordance with the invention, a fibrous product, the

fibers of which may consist entirely of non-proteinaceous 20 fibers which are incapable of felting, is impregnated with the aqueous dispersion of the water-insoluble linear polymer containing the carboxylic groups. The molecular weight of the polymers should be from about 100,000 to about 10 million.

25 The aqueous dispersion is preferably obtained by emulsion polymerization in the presence of an emulsifying agent of at least one monomer containing a carboxyl group, such as acrylic acid, methacrylic acid, and itaconic acid.

30 The emulsifiers or dispersing agents that may be used for preparing the monomeric emulsions before copolymerization or dispersions of the polymer after polymerization may be of anionic or non-ionic type or a mixture of the two types may be used.

35 Suitable anionic dispersing agents include the higher fatty alcohol sulfates, such as sodium lauryl sulfate, alkyl-aryl sulfonates, e.g. sodium or potassium isopropylbenzene sulfonates or isopropyl naphthalene sulfonates, alkali metal higher alkyl sulfosuccinates, e.g. sodium octyl sulfosuccinate, sodium N-methyl-N-palmitoyltaurate, sodium oleyl isothionate, alkali metal salts of alkylarylpolyethoxyethanol sulfates or sulfonates, e.g. sodium t-octylphenoxyphenoxyethoxyethyl sulfate having 1 to 5 oxyethylene units.

40 45 Suitable non-ionic dispersing agents include the following: alkylphenoxyphenoxyethoxyethanols having alkyl groups of about seven to eighteen carbon atoms and 6 to 60 or more oxyethylene units, such as heptylphenoxyphenoxyethoxyethanols, octylphenoxyphenoxyethoxyethanols, methylocetylphenoxyphenoxyethoxyethanols, nonylphenoxyphenoxyethoxyethanols, dodecylphenoxyphenoxyethoxyethanols, and the like; polyethoxyethanol derivatives of methylene linked alkyl phenols; sulfur-containing agents such as those made by condensing 6 to 60 or more moles of ethylene oxide with

50 55 nonyl, dodecyl, tetradecyl, t-dodecyl, and the like mercaptans or with alkylthiophenols having alkyl groups of six to fifteen carbon atoms; ethylene oxide derivatives of long-chained carboxylic acids, such as lauric, myristic, palmitic, oleic, and the like or mixtures of acids such as found in tall oil containing 6 to 60 oxyethylene units per molecule; analogous ethylene oxide condensates of long-chained alcohols, such as octyl, decyl, lauryl, or cetyl alcohols, ethylene oxide derivatives of etherified or esterified polyhydroxy compounds having a hydrophobic hydrocarbon chain, such as sorbitan monostearate containing

60 65 6 to 60 oxyethylene units, etc.; also ethylene oxide condensates of long-chain or branched chain amines, such as dodecylamine, hexadecylamine, and octadecylamine, containing 6 to 60 oxyethylene groups; block copolymers of ethylene oxide and propylene oxide comprising a hydrophobic propylene oxide section combined with one or more hydrophilic ethylene oxide sections.

70 75 The fibers are present in the form of a so-called "non-woven" mat or web in which they are haphazardly distributed. The mat may be formed by carding when the

fibers are of such a character, by virtue of length and flexibility, as to be amenable to the carding operation. Natural fibers like jute, sisal, ramie, hemp, and cotton may be used, as well as many artificial fibers or filaments including rayon, those of cellulose esters such as cellulose acetate, vinyl resin fibers such as those of polyvinyl chloride, copolymers of vinyl chloride with vinyl acetate, vinylidene chloride or acrylonitrile containing a major proportion of vinyl chloride in the polymer molecule, polyacrylonitrile and copolymers of acrylonitrile with vinyl chloride, vinyl acetate, methacrylonitrile, vinyl pyridine, or with mixtures of such comonomers and containing a major proportion from 75% to 95% of acrylonitrile in the copolymer molecule; also condensation polymers such as polyamides of nylon type, polyesters such as ethylene glycol-terephthalate polymers and the like. The thin web or fleece obtained from a single card may be treated in accordance with the present invention, but generally it is necessary and desirable to superpose a plurality of such webs to build up the mat to sufficient thickness for the end use intended, particularly in the making of heat insulation. In building up such a mat, alternate layers of carded webs may be disposed with their fiber orientation directions disposed at 60° or 90° angles with respect to intervening layers.

Mats may also be formed by the deposition of fibers, either natural or artificial, from an air stream. Thus, continuous filaments may be fed to a cutter or breaker which discharges the fibers into the discharge side of a blower. Suitable conduits are provided to guide the fibers to a collecting screen or air-pervious structure for collecting the fibers in the form desired. The screen may be in the form of an endless traveling belt passing through the lower portion of a tower into the upper portion of which the blown fibers are introduced by the conduit work. A suction box may be disposed beneath the upper course of the traveling screen to assist in the deposition of the fibers thereon. Instead of having a traveling flat screen, a stationary formed screen may be used. For example, it may take the form of a hat-shaped cone such as that used in the felt hat-making industry. Alternatively, it may have any other form suitable to produce the desired shape of the fibrous product, such as a rectangular tray. Again, suction may be applied beneath the screen to assist deposition of the fibers thereon.

The fibers and filaments may be formed by direct spraying from a solution or molten mass thereof. This is a conventional procedure for the formation of glass fibers or mineral wool fibers as well as those of nylon or of thermoplastic materials, such as vinyl resins of the type mentioned hereinabove, adapted to be dissolved in a suitable solvent, such as acetone or dimethylformamide, or to be melted. The solution or melt is, of course, directed to suitable nozzles or jet-forming orifices and a high pressure fluid stream, such as of cold or hot air or of inert gases such as nitrogen or even of steam, is directed against the stream or streams of filament-forming material to disrupt them and coagulate them as fibers in the vicinity of the orifices. Electrostatic spinning methods may also be employed for this purpose. As in the case of the use of blowers, the disrupted and dispersed fibers may be directed to the top of a settling tower and be allowed to settle, with the aid of suction devices, upon a suitable traveling or stationary screen at the bottom of the tower. This procedure is adaptable to the production of fibers of siliceous materials such as glass or mineral wool as well as to thermoplastic resin fibers mentioned above.

Another procedure may involve the extrusion of continuous filaments, either from solutions of the filament-forming material or from molten masses thereof, and the cutting or breaking of the filaments to fibers of a predetermined length which may be fed to a hopper at the top of a settling tower into which they may be discharged by conventional feeding devices, and at the bot-

tom of which a traveling or stationary screen may be deposited for collection of the fibers.

The fibers and filaments that may be used in the present invention may be natural or artificial as stated above. The selection of the particular material of which the fiber is made frequently depends upon the use intended of the product. For example, siliceous fibers are extremely valuable in the production of molded articles because of the exceptional strength obtained by their use. However, when the bonded fibrous products are used for filtration purposes, fibers of certain resins may be preferred to provide resistance to attack by acids or alkalies that may be present in the liquids to be filtered. Thus, polymers containing a high percentage of acrylonitrile or of vinyl chloride, or even of such highly halogenated resins as polytetrafluoroethylene or poly(chlorotrifluoroethylene) may be more useful in such cases. For certain purposes, it may be desirable to form the fibrous products from a mixture of fibers of different types. An example is the use of a mixture of thermoplastic fibers of potentially adhesive character with other fibers which lack such potentially adhesive character. A fibrous product comprising such a mixture may be heated to the appropriate temperature to render the potentially adhesive fibers tacky to effect binding of the fibers in the product by this procedure as well as by the binders of the present invention.

The binder of the present invention is applied in the form of an aqueous dispersion which may be produced by the emulsion polymerization of monomers containing carboxyl groups preferably with other monoethylenically unsaturated comonomers. The comonomers may be selected to provide various properties in the binder. Thus, they may provide a soft and flexible binder or they may provide a hard and stiff binder which imparts corresponding stiffness to the bonded fibrous product. Surprisingly, dispersions of copolymers having  $T_g$  values of 50° C. and over can be effectively employed to form coherent-bonded "non-woven" fabrics, even though these dispersions ordinarily do not form continuous films when applied to textile fabrics and dried at temperatures above their respective  $T_g$  values.

Useful comonomers which tend to yield soft and flexible polymers when copolymerized with one of the carboxyl monomers mentioned above are those which yield solid polymers which have a  $T_g$  below 15° to 20° C. The  $T_g$  value referred to is the transition temperature or inflection temperature which is found by plotting the modulus of rigidity against temperature. A convenient method for determining modulus of rigidity and transition temperature is described by I. Williamson, British Plastics 23, 87-90, (September 1950). The  $T_g$  value here used is that determined at 300 kg./cm.<sup>2</sup>.

The polymerizable, neutral, comonomers which form soft, solid polymers in the presence of free radical catalysts include any primary and secondary alkyl acrylates, even with alkyl substituents up to eighteen or more carbon atoms, primary or secondary alkyl methacrylates with alkyl substituents of five to eighteen or more carbon atoms, or other monovinylidene compounds as defined above which are polymerizable below 80° C. with free radical catalysts to form soft solid polymers, including vinyl esters of saturated monocarboxylic esters of over two carbon atoms. The preferred monovinylidene compounds are the stated acrylates and methacrylates and of these the most practical esters are those with alkyl groups of not over 12 carbon atoms.

The preferred monomers which by themselves yield soft polymers may be summarized by the formula



R'

where R' is hydrogen or the methyl group and R\* represents, when R' is methyl, a primary or secondary alkyl group of 5 to 18 carbon atoms, or, when R' is hydrogen,

an alkyl group of not over 18 carbon atoms, or better, of two to 12 carbon atoms.

Typical compounds coming within the above definition are methyl acrylate, ethyl acrylate, propyl acrylate, isopropyl acrylate, butyl acrylate, isobutyl acrylate, sec-butyl acrylate, amyl acrylate, isoamyl acrylate, hexyl acrylate, 2-ethylhexyl acrylate, octyl acrylate, 3,5,5-trimethylhexyl acrylate, decyl acrylate, dodecyl acrylate, cetyl acrylate, octadecyl acrylate, octadecenyl acrylate, n-amyl methacrylate, sec-amyl methacrylate, hexyl methacrylate, 2-ethylbutyl methacrylate, octyl methacrylate, 3,5,5-trimethylhexyl methacrylate, decyl methacrylate, dodecyl methacrylate, octadecyl methacrylate, and butoxyethyl acrylate or methacrylate.

As polymerizable monovinylidene monomers which by themselves form hard polymers, there may be used alkyl methacrylates having alkyl groups of not over four carbon atoms, also tert-amyl methacrylate, tert-butyl or tert-amyl acrylate, cyclohexyl or benzyl acrylate or methacrylate, acrylonitrile, or methacrylonitrile, these constituting a preferred group of the compounds forming hard polymers. Styrene, vinyl chloride, chlorostyrene, vinyl acetate, p-methylstyrene, acrylamide, and methacrylamide also form hard polymers.

Preferred monomers which by themselves form hard polymers may be summarized by the formula



wherein R' is hydrogen or the methyl group and wherein X represents one of the groups —CN, phenyl, methoxyphenyl, and ester-forming groups, —COOR'', wherein R'' is cyclohexyl or, when R' is hydrogen, a tert-alkyl group of four to five carbon atoms, or, when R' is methyl, an alkyl group of one to four carbon atoms. Some typical examples of these have already been named. Other specific compounds are methyl methacrylate, ethyl methacrylate, propyl methacrylate, isopropyl methacrylate, butyl methacrylate, sec-butyl methacrylate, and tert-butyl methacrylate.

It is frequently desirable to copolymerize the carboxyl-containing monomer with a mixture of two or more different comonomers, one or more of which are selected from the hard category just mentioned and another of which is selected from the soft category. An example of this would be a copolymer of 8% to 55% ethyl acrylate, 44% to 90% of methyl methacrylate and from about 3% to 6% of methacrylic acid.

The polymers used as binders of the present invention may also be graft or block copolymers wherein one or more but not all of the monomers are first polymerized and then one or more other monomers are copolymerized with the first polymer obtained. Thus, a carboxyl-containing monomer may first be homopolymerized or copolymerized with one or more, but less than all, of the comonomers to be introduced into the ultimate copolymer, and then the last monomer or monomers are added to the system and copolymerized or grafted on to the first homopolymer or copolymer formed. The same procedure may be used in reverse order to graft the carboxyl-containing units on to a previously formed homopolymer or copolymer of other monomeric units. Again, a plurality of monomeric units may be introduced in succession and the carboxyl-group-containing monomer may be introduced at the beginning, at any intermediate stage or at the end, as desired.

For certain purposes, the copolymers of the present invention having a  $T_1$  of about 30° C. or lower may be preferred. These set on drying at room temperature to bind the fibers with a soft flexible binder bridging the fibers at their points of intersection or intercrossing with a firm grip. Their flexibility adapts the fibrous product to be readily conformed to shaped contours which may be of value in cases where an insulating product or mat is desired to be bent into the shape of a structure

to be covered therewith as in the wrapping of a pipe or cylindrical vessel. Such wrapping can be effected without extensive rupture of the bonds between the fibers and without excessive compacting of the mat, which thereby largely retains its bulky character with numerous small air-spaces and high heat-insulating value and is subsequently rendered permanent by the baking operation. However, for certain purposes, it is preferred to use dispersions of copolymers having a  $T_1$  of 35° C. or higher, such as from 35° to 100° C. In order to effect optimum bonding of the fibers with such a dispersion, it is necessary that the drying be effected at temperatures above the  $T_1$  temperature of the particular copolymer. At lower temperatures, the polymer deposits in particulate form in which the particles are of the order of size of the dispersed resin particles in the aqueous dispersion whereby effective bonding is obtained only where the small particles are lodged within close spacings between the intercrossed fibers. The other particles serve to modify the hand of the web or mat but do not contribute appreciably to the cohesion of the web. By driving the treated fibrous product at temperatures above the  $T_1$  value, fusion or coalescence occurs giving rise to substantial masses adequate in size to bind the fibers at their intersections even when the fibers are separated by relatively large spaces as compared to the size of the original polymer particles in the dispersion. The peculiar advantage of the use of dispersions of polymers, having the elevated  $T_1$  value of at least of about 35° C., is that in the operation of applying the dispersion to the fibrous mass, as by spraying, any excess that is deposited on the walls of the spraying chamber dries at the prevailing room temperature below 35° C. to discrete particles or a powder which is readily removed from the equipment merely by brushing. To take advantage of this properly, care is taken to avoid any substantial elevation of the temperature in the application equipment, such as the spraying equipment or chamber, appreciably above room temperature in cases where the  $T_1$  value of the copolymer is in the neighborhood of 35° C. Of course, when higher  $T_1$  values of 55° to 100° C. characterize the polymer, considerable elevation of the temperature in the spraying equipment may be present without encountering coalescence in the excess material deposited in the walls of the equipment, provided the temperature surrounding such equipment does not approach too closely (say within 10° C.) the temperature of the  $T_1$  value of the particular polymer involved.

In the preparation of bonded fibrous products of the present invention, which are intended to serve as preforms in the making of molded products, the use of polymers having higher  $T_1$  values also has the advantage that the preform is much stiffer in character and encounters less risk of disturbance of the fibers during the handling of the preform in preparing it for the molding operation per se.

The dispersions adapted to be used as the binder-applying medium of the present invention are most advantageously prepared by emulsifying with a dispersing agent and polymerizing, preferably under the influence of a free radical catalyst, a mixture of the monomers of which at least one-half percent is a carboxyl-containing monomer.

Anionic and non-ionic emulsifiers or dispersing agents may be used. Less advantageously, water-insoluble polymers comprising at least 0.5% of carboxyl-containing monomeric units produced in any other way may be dispersed in water by means of suitable dispersing agents.

The dispersions may contain as little as 1% and as much as 60% of the resinous copolymer on a weight basis. It is, however, more practical—hence preferred—to produce dispersions which contain about 30% to 50% resin-solids. Generally, the dispersion is diluted to 1% to 35%, and preferably 2% to 30%, resin content at

which it is readily adapted to be applied as by spraying, dipping, or by transfer rolls.

The binder dispersion may be applied to the dry fibers after the formation or deposition of the web or mat so as to penetrate partially into or completely through the interior of the fibrous products. Alternatively, the binder dispersion may be applied to the fibers as they fall through the settling chamber to their point of deposition. This is advantageously obtained by spraying the binder dispersion into the settling chamber at some intermediate point between the top and the bottom thereof. By so spraying the fibers as they descend to the point of collection it is possible to effect a thorough distribution of the binder among the fibers before they are collected into the product. In the production of certain fibrous products wherein a hot molten mass of a polymer, such as nylon or a fused siliceous mass or glass, is disrupted by jets of heated air or steam, the binder dispersion may be sprayed directly on the fibers while still hot and very shortly before their deposition so that quickly after deposition the binder is set and bonds the fibers in proper relationship. Preferably, however, application of the binder dispersion to the fibrous product is made at room temperature to facilitate cleaning of the apparatus associated with the application of the binder dispersion. The binder dispersion may be applied to one or both surfaces of the fibrous product or it may be distributed through the interior as well. While the binder may be applied in powdered form in each of the situations just mentioned, in all cases application of the aqueous dispersion is preferred.

While chemical reaction probably occurs between the binders of the present invention and fibers, such as those of cellulosic type, which contain reactive groups, it is not intended that the invention should be limited to this theory operation.

The binder of the present invention may be applied in conjunction with other binders. For example, another type of binder, such as glue or resin-forming condensates, especially aminoplasts such as urea-formaldehyde, melamine-formaldehyde and the like, may be applied either to the interior or to the external surfaces of the fibrous product while the binder of the present invention is applied to the external surfaces or to the interior of such products. Similarly, the use of potentially adhesive fibers within the fibrous product may also be resorted to in conjunction with the use of a binder of the present invention. The aqueous copolymer dispersion may also contain dissolved therein a water-soluble thermosetting condensation product, especially the aminoplasts, namely the low molecular weight or monomeric reaction products of an aldehyde, and especially formaldehyde with urea, thiourea, biuret, or other homologues or derivatives thereof, such as N,N-ethyleneurea, N,N'-ethyleneurea, N,N'-dimethylurea, N,N'-diethylurea, N,N'-dimethoxymethylurea, N,N-dimethoxymethylurea, N,N'-diethoxymethylurea, tetramethoxymethylurea, tetraethoxymethylurea. Similar reaction products of formaldehyde with triazines, such as melamine may also be employed, such as N,N-dimethylmelamine and alcohol-modified-melamine-formaldehyde thermosetting resin condensates, e.g. of methyl and ethyl alcohols, for example, dimethoxymethyl-monomethylolmelamine.

The auxiliary aminoplast binder may be used in an amount up to 25% by weight of the weight of polymer containing carboxyl groups, 2 to 11% being preferably employed when the combination binder system is used. The use of an auxiliary aminoplast with the carboxyl-containing polymers of the present invention serves to modify the hand, and frequently increases the strength and resistance to creasing, wrinkling, and crushing.

When an aminoplast binder is used in conjunction with the polymer containing carboxyl groups, there may be introduced into the system either into the aqueous dispersion of the polymer or by separate application to

the non-woven fibrous mat or web before or after application of the aqueous dispersion of the polymer, a catalyst for accelerating the curing of the copolymer/aminoplast binder. The catalyst may be used in an amount up to 5 to 2%, preferably about 1/2 to 1% on the weight of the aminoplast. The catalyst used may be selected to avoid excessive deterioration of the fibers used in the particular fibrous product, but it is in any case an acidic or potentially acidic material, the latter serving as a latent catalyst and liberating acid on heating. For example, when cellulosic fibers are employed, a latent ammonium salt, such as ammonium chloride or diammonium phosphate or a latent amine hydrochloride salt, may be employed such as the hydrochloride of triethanolamine, monoethanolamine, diethylamine, and so on.

If desired, the aqueous dispersion of the polymer containing carboxylic units may also contain a wetting agent to assist penetration of the fibrous web or mat to which it is applied, and it may contain either a foaming agent 10 to provide the binder in a foamed condition in the final product or it may contain a defoamer when the ingredients of the aqueous dispersion have a tendency to give rise to foaming, and in a particular case such foaming is undesirable. The conventional wetting agents, such as 20 the sodium salt of diethylsulfosuccinate may be used and the conventional foaming and defoaming agents may be employed, such as sodium soaps, including sodium oleate for foaming and octyl alcohol or certain silicones for defoaming.

Generally, the proportion of the binder of the present invention to the weight of the fiber component of the fibrous product may vary widely depending on the character of the product desired. For the production of preforms, intended to be converted into molded articles, it 30 is preferred to employ from 2 to 10% of the binder of the present invention based on the weight of fibers. In the production of insulation masses, the amount of binder employed may fall in the lower part of the range just specified if the binder is applied primarily adjacent to the 40 surface or surfaces of the product or if it is applied in conjunction with other binders. The aqueous dispersion of the polymer containing the carboxyl groups is generally applied at a concentration of 2 to 60% solids and preferably at a concentration of 20 to 40% binder solids by 45 weight.

The fibrous product of non-woven character may contain from 2 to 400% by weight of binder on the weight of the fibers depending on the purpose for which the product is to be used. When the binder is to serve mainly 50 to bond the fibers together to form a coherent unitary structure in which the maximum porosity is retained in conjunction with a minimum change of natural fiber hand, there may be employed from 2 to 50% by weight of binder solids on fiber, the lower proportion of course 55 giving the maximum porosity possible and providing a minimum change in the natural fiber hand although even with the larger proportion in this range, the porosity is mainly retained and the fiber hand is still evident. The products thus obtained are quite useful for many 60 sanitary uses such as table napkins, bibs, table cloths, sanitary napkin covers, disposable diapers, disposable sheets, and surgical dressings and compresses. It is characteristic of the binder applied in the proportions just stated that there is relatively little or no "window 65 paning," that is the interstices between fibers is left open leaving a highly porous bulky product. Of course, the density of the product can be effected or modified by the application of pressure to varying extents prior to or, in many cases, even after the curing of the product.

70 Fibrous products of non-woven character using from 40 to 150% by weight of the binder of the present invention on the weight of the fiber are generally quite useful for garment uses to provide interlining fabrics for coats, dresses, and so on, or to provide outer wearing apparel fabrics, such as blouses, skirts, shirts, etc. The garments

made of these fabrics need no ironing or pressing to restore their appearance, shape, and hand after hand washing, machine laundering, and drying operation. Besides the general household and apparel uses mentioned above, fibrous products of the invention, in which 2 to 100% by weight of binder on the weight of fiber is employed, find many light industrial uses as wiping cloths, lining materials for packaging as filters, and packings and gaskets for industrial machinery.

Fibrous products of the present invention in which 100 to 400% by weight of the binder on the weight of fiber is used are especially useful for heavy industrial uses where durability and resistance to wear are desired, such as in industrial gaskets, packings, filters, and so on. The products containing 20 to 200% of the binder of the present invention on the weight of the fiber are useful as laminating layers, either as interlayers or backing sheets in conjunction with plastic films and sheets as of polyethylene, nylon, and so on, or in conjunction with textile fabrics of woven, braided, knitted, knotted, or felted character.

It is essential that the drying of the treated fibrous product, that is the fibrous product carrying the binder dispersion, be effected at a temperature above the  $T_1$  of the binder copolymer in order to effect proper coalescence and bonding of the fibers. As pointed out above, if the  $T_1$  of the copolymer is about 30° C. or lower, no special heating is necessary to effect bonding, but it may be advantageous to accelerate the drying of the binder to the set condition. To render the binder infusible, curing at elevated temperatures is effected. Curing temperatures may be as high as 400° C. for setting the binder, but preferably are in the range from about 110° C. to 350° C. The curing serves to render the binder insoluble and infusible and, as stated hereinabove, may be assisted by the use of an acidic catalyst where an aminoplast is used.

As pointed out hereinbefore, the application of the polymers containing carboxyl groups is adapted to provide fibrous products having a wide range of characteristics. When the binder is present in an amount of about 2 to 50% on the weight of the fibers in the fibrous product, the latter retains a textile hand and can have either a soft or a stiff texture depending on the proportion of carboxyl groups in the polymer and the characteristics of any comonomers used in making it. Using polymers containing ½ to 10% of units containing carboxyl groups in conjunction with such comonomers as result in providing a  $T_1$  value of the copolymer of 20° C. or less and preferably not over 5° C., a soft resilient texture is obtained in conjunction with a textile feel or hand and the cured product is quite resistant to laundering, dry-cleaning and spotting to various chemicals and heat. In all of the fibrous products previously mentioned, where the binder may be present in the proportion of 2 to 50% as in the products just mentioned or in larger proportions up to 400% on the weight of the fiber, the products are characterized by freedom from discoloration and excellent resistance to laundering, dry-cleaning and spotting, to various chemicals, and heat as in ironing, good adhesion of the binder to the fibers, and durability of any embossed pattern.

The binder of the present invention is essentially colorless and has the advantage that it undergoes no discoloration at the elevated temperature needed for the drying or baking of the fibrous products or even for the formation of molded articles with the fibrous products of the present invention used as preforms and ultimately occurring as a reinforcing component in the molded article. The binder of the present invention is resistant to flow at elevated temperatures so a thermoplastic or thermosetting resin can be applied and the composite thereby obtained can be molded at elevated temperature without appreciably disturbing the disposition of fibers in the mass. Similarly, the binder is insoluble in water and organic solvents so that the presence of such materials during sub-

sequent treatment as in molding cannot disturb the disposition of fibers. Consequently, there is no "washing" of fibers in the preform with accompanying tendency to form resin-rich areas and fiber-rich areas in the molded article giving rise to such non-uniformity which tends to cause cracking or crazing in the molded articles and resulting weakness in the reinforced structure.

All of these properties render the binder outstandingly valuable in connection with siliceous fibers, such as those of glass or mineral wool, in the production of preforms adapted to be used for forming molded articles. The siliceous fibers are strongly bonded together by means of the binders of the present invention and especially those having a  $T_1$  temperature above 35° C. and yet the binder is of such character as not to prevent proper integration of the siliceous fibers within the mass of molding resin. In the molded products, the presence of the binder has no adverse effect either on the appearance or the strength of the final articles. While molding resins or resin-forming materials of numerous thermoplastic and thermosetting types may be employed, the use of thermosetting types of polyesters is particularly advantageous. Such a resin-forming material may comprise an unsaturated polyester (such as a polyester of mixed maleic acid and phthalic acid (in a 50-50 molar ratio) with a glycol, such as propylene glycol) dissolved in styrene or other copolymerizable monoethylenically unsaturated monomers having solvent properties for the low condensed polyester. Most binders heretofore used in the preforms become discolored during the molding operation and interfere with the penetration of the molding resin, especially when it is of a polyester type, so that the fused resin is poorly bonded to the portions of the fibers coated by the binder which in turn is manifested by a reduced transparency and corresponding lack of continuity and homogeneity. The binder of the present invention is resistant to such discoloration. In addition, it does not interfere with the penetration of the resin-forming material to the fibers of the preform during the molding operation. This provides excellent transparency and a high degree of homogeneity and continuity in the product. Also, the binders of the present invention having the higher  $T_1$  values and accompanying higher stiffness assure the maintenance of the distribution of the fibers during the handling of the preform up to the molding operation.

The fibrous products of the present invention are capable of numerous uses, many of which have been mentioned above. Thus, the fibrous mats bonded with the improved binders of the present invention may serve as heat or sound insulation materials, as filters for air systems or liquid systems, as permeable membranes as in storage batteries or electrolytic condensers, as cushioning or padding materials for upholstering purposes and so forth.

As pointed out hereinabove, fibrous mats or fabrics of siliceous fibers are extremely valuable as reinforcements for molded products using the bonded fibrous mat or fabric as a preform with appropriate molding powders or syrups. For example, the bonded mat or the bonded laminar fabric assembly may be introduced into a closed mold system with an appropriate amount of a thermosetting resin powder or liquid, such as of resin-forming condensates of urea-formaldehyde, melamine-formaldehyde, phenol-formaldehyde or polyesters, such as those described in U.S. Patents 2,255,313 and 2,607,756. From 5 to 45% by weight of the molded article may be composed of the reinforcing fiber network when a mat is used as the preform or, in the case of a fabric reinforcement, from 5 to 65% by weight of the molded product may consist of the composite of bonded fabric laminations.

Instead of using a thermosetting resin-forming material as the molding resin, there may be used thermoplastic types of resins such as the vinyl or acrylic types of resins. For example, polymers and copolymers of vinyl acetate, vinyl chloride, acrylonitrile, styrene, acrylic, and methacrylic acid esters; e.g. the methyl, ethyl, propyl

or butyl esters thereof, and so on. Advantageously, a polymer or copolymer may be dissolved in its corresponding monomer or mixture of monomers to provide a solution that may readily be introduced into the mold.

The following examples are illustrative of the fibrous products and the methods for making them in accordance with the present invention and parts and percentages are by weight unless otherwise indicated:

*Example 1*

(a) A 75/25 viscose (3 denier, 1 inch staple)/bleached cotton (middling,  $1\frac{1}{16}$  inch) carded web weighing about 0.75 ounce/square yard is impregnated with an aqueous dispersion containing per 100 parts:

25.0 parts of the ammonium salt of a 66% ethyl acrylate, 32.7% methyl methacrylate, and 1.3% methacrylic acid emulsion copolymer

2 parts of t-octylphenoxypolyethoxyethanol containing about 35 oxyethylene units (emulsifier and dispersing agent)

0.4 part of octylphenoxyethoxysodiumsulfate (wetting agent)

0.1 part silicone antifoam

at a wet pick-up of about 600% on the weight of the fibers. The web is dried 1.5 minutes at 225° F., and cured 1.5 minutes at 350° F. The resulting non-woven fabric is about 33/67 fiber/binder. It is highly porous and has a soft and resilient feel.

(b) The procedure of part (a) is repeated with Pyrex glass fibers, except that the carded web weighed  $\frac{1}{2}$  ounce per square yard and impregnation with the aqueous dispersion is effected at a wet pick-up of 300%, giving a weight ratio of 53/47 fiber to binder in the final fabric which is extremely porous and soft yet coherent.

*Example 2*

The procedure of Example 1(a) is repeated using a similar aqueous dispersion containing 25.0 parts of the sodium salt of an emulsion copolymer of 85% of ethyl acrylate with 15% of methyl methacrylate, the acrylate groups having been hydrolyzed to introduce about 2% of acrylic acid into the copolymer. A porous, soft and coherent non-woven web is obtained.

*Example 3*

The procedure of Example 1(a) is repeated using a similar aqueous dispersion containing 25.0 parts of the sodium salt of an emulsion copolymer of 87% of ethyl acrylate, 10.5% of methyl methacrylate, and 2.5% of itaconic acid. An exceptionally well-bonded non-woven web is obtained that is highly resistant to solvents and heat.

*Example 4*

The procedure of Example 1(a) is repeated using a similar aqueous dispersion containing 25.0 parts of the sodium salt of an emulsion copolymer of 97.5% of ethyl acrylate and 2.5% of itaconic acid. A coherent web like that of Example 3 but with a softer hand is obtained.

*Example 5*

A 50/50 white nylon/disperse-dyed bright acetate (both fibers 3 denier, 1.5 inch staple) random web obtained by air-deposition weighing about 1.5 oz./sq. yd. is impregnated with an aqueous dispersion containing per 100 parts:

27.0 parts of the sodium salt of a copolymer of 10% ethyl acrylate, 89.5% methyl methacrylate, and 0.5% of methacrylic acid

2 parts of t-octylphenoxypolyethoxyethanol containing about 35 oxyethylene units (emulsifier and dispersing agent)

3.0 parts of dimethylol-N,N'-ethyleneurea

0.5 part of ammonium chloride

0.5 part of octylphenoxyethoxysodiumsulfate (wetting agent)

0.1 part of silicone antifoam

at about 300% wet pick-up. The web is dried 1.5 minutes at 225° F., cured six minutes at 350° F. Resultant non-woven fabric is ca. 55/45 fiber/binder. It is quite porous and has an essentially textile hand. After washing and drying, no ironing or pressing is needed to restore the shape, appearance, or hand of garments made of the fabric.

*Example 6*

A 50/50 white viscose/dyed Acrilan (polymer of about 85% to 90% acrylonitrile) (both fibers 3 denier, 1.5 inch staple) random web obtained by air-deposition weighing about 1.75 oz./sq. yd. is impregnated with an aqueous dispersion containing per 100 parts:

27 parts of the triethylamine salt of a copolymer of 7% acrylic acid and 93% of n-butyl acrylate

2 parts of t-octylphenoxypolyethoxyethanol containing about 35 oxyethylene units (emulsifier and dispersing agent)

3.0 parts of urea/formaldehyde/methanol condensate

0.5 part of diammonium phosphate

0.5 part of octylphenoxyethoxysodiumsulfate (wetting agent)

0.02 part of silicone antifoam

at ca. 300% wet pick-up. Dried 1.5 min. at 225° F., cured five min. at 350° F. Product: 55/45, fiber/binder; good coherence, porous, soft, textile hand.

It is to be understood that changes and variations may be made without departing from the spirit and scope of the invention as defined in the appended claims.

35 We claim:

1. As an article of manufacture, a non-woven fibrous product in which the fibers are distributed in random array, the fibers of which are predominantly fibers which are incapable of felting selected from the group consisting of cellulosic fibers, nylon fibers, vinyl resin fibers, poly(ethylene glycol terephthalate) fibers, and mixtures thereof, fibers in the product being bonded together by a binder substantially uniformly distributed through the thickness of the product and comprising a water-insoluble emulsion copolymer of monoethylenically unsaturated monomeric units comprising 0.5 to 10% by weight of a compound selected from the group consisting of acrylic acid, methacrylic acid, itaconic acid, and ammonium, amine, and alkali metal salts thereof with at least one ester of an acid selected from the group consisting of acrylic acid and methacrylic acid with an alcohol having 1 to 12 carbon atoms, said copolymer being cross-linked to an insoluble condition whereby the product is substantially resistant to dry-cleaning, the amount of binder being from 2 to 400% of the weight of fibers in the product, and the molecular weight of the copolymer being at least 100,000.

2. As an article of manufacture, a non-woven fibrous product in which the fibers are distributed in random array, the fibers of which comprise a predominant proportion of cellulosic fibers which are incapable of felting, fibers in the product being bonded together by a binder substantially uniformly distributed through the thickness of the product and comprising a water-insoluble emulsion copolymer of 0.5 to 10% by weight of a compound selected from the group consisting of acrylic, methacrylic, and itaconic acids, and ammonium, amine, and alkali metal salts thereof with at least one ester of an acid selected from the group consisting of acrylic acid and methacrylic acid with an alcohol having 1 to 12 carbon atoms, said copolymer being cross-linked to an insoluble condition whereby the product is substantially resistant to dry-cleaning, the amount of binder being from 2 to 400% of the weight of fibers in the product, and the molecular weight of the copolymer being at least 100,000.

3. As an article of manufacture, a non-woven fibrous product in which the fibers are distributed in random array, the fibers of which are predominantly fibers which are incapable of felting selected from the group consisting of cellulosic fibers, nylon fibers, vinyl resin fibers, poly(ethylene glycol terephthalate) fibers, and mixtures thereof, fibers in the product being bonded together by a binder substantially uniformly distributed through the thickness of the product and comprising the reaction product of (1) an aminoplast selected from the group consisting of condensation products of formaldehyde with urea, N,N-ethyleneurea, and melamine and (2) a water-insoluble emulsion copolymer of monoethylenically unsaturated monomeric units comprising 0.5 to 10% by weight of a compound selected from the group consisting of acrylic acid, methacrylic acid, itaconic acid, and ammonium, amine, and alkali metal salts thereof with at least one ester of an acid selected from the group consisting of acrylic acid and methacrylic acid with an alcohol having 1 to 12 carbon atoms, said product being substantially resistant to laundering and dry-cleaning, the amount of aminoplast being from 2 to 25% by weight of the copolymer and the amount of binder being from 2 to 400% of the weight of fibers in the product, and the molecular weight of the copolymer being at least 100,000.

4. As an article of manufacture, a non-woven fibrous product in which the fibers are distributed in random array, the fibers of which comprise a proportion of cellulosic fibers, fibers in the product being bonded together by a binder substantially uniformly distributed through the thickness of the product and comprising the heat-cured product of (1) an aminoplast selected from the group consisting of condensation products of formaldehyde with urea, N,N-ethyleneurea, and melamine and (2) a water-insoluble emulsion copolymer of 0.5 to 10% by weight of a compound selected from the group consisting of acrylic, methacrylic, and itaconic acids, and ammonium, amine, and alkali metal salts thereof with at least one ester of an acid selected from the group consisting of acrylic acid and methacrylic acid with an alcohol having 1 to 12 carbon atoms, said product being substantially resistant to laundering and dry-cleaning, the amount of aminoplast being from 2 to 25% by weight of the copolymer and the amount of binder being from 2 to 400% by weight of fibers in the product, and the molecular weight of the copolymer being at least 100,000.

5. A product as defined in claim 4 in which the copolymer is an alkali metal salt of a copolymer of 0.5 to 10% of acrylic acid with ethyl acrylate and methyl methacrylate.

6. A product as defined in claim 4 in which the copolymer is an ammonium salt of a copolymer of 0.5 to 10% of methacrylic acid with ethyl acrylate and methyl methacrylate.

7. A product as defined in claim 4 in which the copolymer is an ammonium salt of a copolymer of 0.5 to 10% of methacrylic acid with ethyl acrylate and methyl methacrylate and the aminoplast comprises dimethylol-N,N'-ethyleneurea.

8. A product as defined in claim 4 in which the copolymer is an ammonium salt of a copolymer of 0.5 to 10% of methacrylic acid with ethyl acrylate and methyl methacrylate and the aminoplast comprises a condensation product of melamine and formaldehyde.

9. As an article of manufacture, a non-woven fibrous product in which the fibers are distributed in random array, the fibers of which are predominantly fibers which are incapable of felting selected from the group consisting of cellulosic fibers, nylon fibers, vinyl resin fibers, poly(ethylene glycol terephthalate) fibers, and mixtures thereof, fibers in the product being bonded together by a binder substantially uniformly distributed through the thickness of the product and comprising a water-insoluble emulsion copolymer of monoethylenically unsaturated monomeric units comprising 0.5 to 10% by weight of a

5

10

15

20

25

30

35

40

45

50

55

60

65

70

75

compound selected from the group consisting of itaconic acid, and ammonium, amine, and alkali salts thereof with at least one ester of an acid selected from the group consisting of acrylic acid and methacrylic acid with an alcohol having 1 to 12 carbon atoms, said copolymer being cross-linked to an insoluble condition whereby the product is substantially resistant to laundering and dry-cleaning, the amount of binder being from 2 to 400% of the weight of fibers in the product, and the molecular weight of the copolymer being at least 100,000.

10. As an article of manufacture, a non-woven fibrous product in which the fibers are distributed in random array, the fibers of which comprise cellulosic fibers, fibers in the product being bonded together by a binder substantially uniformly distributed through the thickness of the product and comprising a water-insoluble emulsion copolymer, having a molecular weight of at least 100,000, of 0.5 to 10% by weight of a compound selected from the group consisting of itaconic acid, and ammonium, amine, and alkali metal salts thereof with at least one ester of an acid selected from the group consisting of acrylic acid and methacrylic acid with an alcohol having 1 to 12 carbon atoms, said copolymer being cross-linked to an insoluble condition whereby the product is substantially resistant to laundering and dry-cleaning, the amount of binder being from 2 to 400% of the weight of fibers in the product.

11. A product as defined in claim 10 in which the copolymer is an alkali metal salt of a copolymer of 0.5 to 10% of itaconic acid with ethyl acrylate and methyl methacrylate.

12. As an article of manufacture, a non-woven fibrous product in which fibers selected from the group consisting of cellulosic fibers, nylon fibers, vinyl resin fibers, poly(ethylene glycol terephthalate) fibers, and mixtures thereof are distributed in random array, fibers in the product being bonded together by a binder substantially uniformly distributed through the thickness of the product and comprising a water-insoluble alkali metal salt of an emulsion copolymer, having a molecular weight of at least 100,000, of 0.5 to 10% of itaconic acid with ethyl acrylate and methyl methacrylate, said product being substantially resistant to laundering and dry-cleaning, the amount of binder being from 2 to 400% of the weight of fibers in the product.

13. A process of making a non-woven fabric which comprises associating, in random array within a web or mat, a mass of fibers comprising a predominant proportion of fibers which are incapable of felting selected from the group consisting of cellulosic fibers, nylon fibers, vinyl resin fibers, poly(ethylene glycol terephthalate) fibers, and mixtures thereof, bringing into contact with the fibers, substantially uniformly through the fibrous mass, an aqueous dispersion containing 2 to 60% by weight of a water-insoluble emulsion copolymer, having a molecular weight of at least 100,000, of monoethylenically unsaturated monomeric units comprising 0.5 to 10% by weight of a compound selected from the group consisting of acrylic, methacrylic, and itaconic acids, and ammonium, amine, and alkali metal salts thereof with at least one ester of an acid selected from the group consisting of acrylic acid and methacrylic acid with an alcohol having 1 to 12 carbon atoms, and drying the fibrous mass containing from 2 to 400%, based on the weight of

fibers, of the copolymer at a temperature above the  $T_g$  of the copolymer to effect fusion of the copolymer and bonding of the fibers thereby, and heating the dried fibrous product at a temperature of  $110^\circ$  to  $350^\circ$  C. to insolubilize the binder with respect to dry-cleaning solvents.

14. A process as defined in claim 13 in which the aqueous dispersion also contains dissolved therein an aminoplast condensate in an amount of 2 to 25% by weight of the copolymer.

15. A process of making a non-woven fabric which

comprises associating, in random array within a web or mat, a mass of fibers comprising a predominant proportion of fibers which are incapable of felting selected from the group consisting of cellulosic fibers, nylon fibers, vinyl resin fibers, poly(ethylene glycol terephthalate) fibers, and mixtures thereof, bringing into contact with the fibers, substantially uniformly through the fibrous mass, an aqueous dispersion containing 2 to 60% by weight of a water-insoluble emulsion copolymer, having a molecular weight of at least 100,000, of monoethylenically unsaturated monomeric units comprising 0.5 to 10% by weight of a compound selected from the group consisting of itaconic acid, and ammonium, amine, and alkali metal salts thereof with at least one ester of an acid selected from the group consisting of acrylic acid and methacrylic acid with an alcohol having 1 to 12 carbon atoms, and drying the fibrous mass containing from 2 to 400%, based on the weight of fibers, of the copolymer at a temperature above the  $T_g$  of the copolymer to effect fusion of the copolymer and bonding of the fibers thereby, and heating the dried fibrous product at a temperature of 110° to 350° C. to insolubilize the binder with respect to dry-cleaning solvents and laundering.

## References Cited in the file of this patent

## UNITED STATES PATENTS

|    |           |                    |                |
|----|-----------|--------------------|----------------|
| 5  | 2,256,034 | Nottebohm          | Sept. 16, 1941 |
|    | 2,338,960 | Nottebohm          | Jan. 11, 1944  |
|    | 2,516,836 | Drechsel           | Aug. 1, 1950   |
|    | 2,531,408 | D'Alelio           | Nov. 28, 1950  |
|    | 2,653,140 | Allenby et al.     | Sept. 22, 1953 |
| 10 | 2,686,772 | Bortnick           | Aug. 17, 1954  |
|    | 2,694,695 | Bortnick           | Nov. 16, 1954  |
|    | 2,719,072 | Kine               | Sept. 27, 1955 |
|    | 2,719,795 | Nottebohm          | Oct. 4, 1955   |
|    | 2,719,803 | Nottebohm          | Oct. 4, 1955   |
|    | 2,719,806 | Nottebohm          | Oct. 4, 1955   |
| 15 | 2,719,832 | Craemer et al.     | Oct. 4, 1955   |
|    | 2,726,230 | Carlson            | Dec. 6, 1955   |
|    | 2,727,015 | Auten et al.       | Dec. 13, 1955  |
|    | 2,760,945 | Bodenschatz et al. | Aug. 28, 1956  |
|    | 2,790,736 | McLaughlin et al.  | Apr. 30, 1957  |
| 20 | 2,823,142 | Sumner et al.      | Feb. 11, 1958  |

## OTHER REFERENCES

- Ser. No. 202,136, Nottebohm (A.P.C.), published May 11, 1943.  
 Ser. No. 306,031, Nottebohm (A.P.C.), published May 11, 1943.